

A. W. SCHORGER.  
DRY CELL.  
APPLICATION FILED JAN. 25, 1919.  
**1,370,052.**

Patented Mar. 1, 1921.

Fig. 1.



Fig. 2.



INVENTOR  
Arlie W. Schorger

BY

Perrine Davis Marvin & Edmunds  
ATTORNEYS

# UNITED STATES PATENT OFFICE.

ARLIE WILLIAM SCHORGER, OF MADISON, WISCONSIN, ASSIGNOR TO BURGESS BATTERY COMPANY, OF MADISON, WISCONSIN, A CORPORATION OF WISCONSIN.

## DRY CELL.

1,370,052.

Specification of Letters Patent.

Patented Mar. 1, 1921.

Original application filed November 19, 1918, Serial No. 263,119. Divided and this application filed January 25, 1919. Serial No. 273,020.

To all whom it may concern:

Be it known that I, ARLIE W. SCHORGER, a citizen of the United States, residing at Madison, in the county of Dane and State 5 of Wisconsin, have invented certain new and useful Improvements in Dry Cells, (division of application filed Nov. 19, 1918, Ser. No. 263,119;) and I do hereby declare the following to be a full, clear, and exact description of the invention, such as will enable others skilled in the art to which it appertains to make and use the same.

Electric dry cells can be roughly grouped into two general classes. In the first class, 15 as illustrated, for instance, in Burgess and Hambuechen U. S. Patent Number 1,032,529, issued July 16, 1912, the zinc can is lined with paper or other equivalent bibulous material and the so-called "mix" consisting of carbonaceous material, manganese-dioxid and the usual salts and moisture is tamped about a carbon rod, thereby forming the cathode which is spaced from the zinc or anode by the layer of moistened 25 paper.

In the second class, the mix, before its introduction into the zinc can, is molded about the carbon rod to form a so-called "core" which, though fragile, is nevertheless 30 capable of manipulation on a factory basis. A suitable apparatus for thus molding the moist mix about a carbon rod is disclosed in U. S. patent to Hambuechen Number 1,232,297, issued July 3, 1917. The core so 35 formed is next wrapped about with gauze, cheesecloth or the like, held in place by rubber bands or by a wrapping of thread, as disclosed in Burgess U. S. Patent Number 1,162,449, issued November 30, 1915.

40 The wrapped core is then introduced into the zinc can, and an electrolyte in the form of a gelatinizable paste is poured into the annular space separating the core from the wall of the zinc can. It is quite customary 45 to gelatinize this paste by a cooking operation, and the gauze wrapping prevents disintegration and washing away of the molded mix during the cooking, and, of course, prevents the mix from crumbling away and 50 dropping into contact with the zinc during the preceding operation of assembly. These cells are ordinarily said to be of the "bag type" because the gauze wrapping forms in effect a bibulous bag to hold the mix in posi-

tion during assembly and during cooking 55 of the gelatinizable electrolyte. After the electrolyte has been hardened to a jelly-like consistency, the gauze wrapping is no longer essential, and in fact its presence in the cell presents some objections, as will be well 60 understood by those skilled in the art.

The present invention relates to galvanic cells of the bag type and has as one of its objects the elimination of the gauze bag and the substitution for it during assembly of 65 a hard, thin and porous covering preferably put on by dipping the molded core into a magma such as a mixture of plaster of Paris and water.

It is a further object of the present invention to simplify and cheapen the process of manufacture by eliminating the expensive gauze bag and the tedious and expensive operations of wrapping the core with the gauze and binding it in place with a wrapping of 75 thread or the like.

It is a further object to produce a finished battery of the bag type of high output, low internal resistance and good shelf life, as the results of this new method of 80 production and this new structural arrangement of the core or cathode of the cell.

The accompanying drawing, Figure 1 illustrates, somewhat diagrammatically, a cell constructed in accordance with the present invention. Fig. 2 shows a modification.

In the drawing, 1 is the zinc can serving as anode and also as a fluid tight container for the other elements of the cell; 2 is the gelatinized electrolyte; 3 is a carbon rod 90 enveloped in the molded mix 4 of carbonaceous material, manganese dioxid, etc., and 5 is the envelop or bag of hardened plaster dip. The carbon rod may have a brass terminal cap 6, a pitch seal 7, a cardboard 95 washer 8, and an air space 9, as is usual in dry cell construction, and may be of any desired size, as, for instance, six inches high to conform with standard telephone practice, or of a much smaller size for use in 100 battery hand lamps and like novelties.

The process of assembling the component parts to make a cell of this construction is as follows: The mix 4 is molded about the carbon rod 3 in a suitable tamping machine, 105 as of the construction shown in Hambuechen Patent 1,232,297, and the fragile core thus formed is dipped into a magma, preferably

consisting essentially of a suspension of plaster, such as plaster of Paris, in water, so that after dipping, the core will be covered with a thin film of the dip which on 5 hardening will form an envelop for the molded part of the core. The film of dip can be relatively thin and will harden quickly to form a substantially continuous, uniform membrane or bibulous envelop. As 10 a factory expedient, the dip may be allowed to harden while the cores rest on a greased plate or on a smooth bed of sand. This prevents sticking to the support, and when sand is used, a certain amount clings to the bottom 15 of the core, as illustrated diagrammatically in the drawing at 10, where the core rests on the zinc bottom of the can. These particles of sand then act to separate and insulate the core from the bottom of the zinc 20 can and obviate the need for covering the zinc bottom with a disk of paraffin paper, as is common practice, or the need for impregnating the lower portion of the core with paraffin, as described in Burgess Patent 25 1,162,449. There is thus obtained some saving in labor and some economy in material.

After the core has become thoroughly hardened on the greased plate or on the bed of sand, it is introduced into its zinc can and 30 the electrolyte is poured into the annular space between the core and the zinc can, in accordance with the usual practice of assembling bag type cells. The gelatinizable electrolyte may consist of a mixture of 35 cereals and zinc and ammonium chlorids, capable of gelatinization on heating, though I prefer to use a water solution containing about 25.5% of cereals, say, cornstarch and cornmeal, and 36.7% of zinc and ammonium 40 chlorids, all at a temperature considerably lower than room temperature for this mixture, though not original with me, is of such a character as to function in advantageous manner as a part of the cell, more particularly 45 because it gelatinizes without the need for a subsequent cooking operation.

The magma into which the cores are dipped to form the film which subsequently hardens to a coherent bibulous envelop may 50 vary in composition, and there are herein-after described several which are suitable, and some of which offer special advantages.

*Plaster only.*—A mixture of water and plaster in suspension forms a suitable dip. 55 Thus I may use 225 grams plaster of Paris and 250 grams of water. A core dipped into such a suspension takes on a film which on drying hardens into a porous, continuous, strong cup or envelop completely surrounding the core. The proportion of plaster of Paris to water may be varied through relatively wide limits in order to vary the thickness of the hardened film, for the thinner the magma the thinner will be the film produced on the core. Another suitable mix-

ture consists of 20 grams zinc oxid; 20 grams zinc chlorid, and 10 grams water. Also, there may be used 20 grams magnesium oxid; 20 grams magnesium chlorid, and 150 grams water.

With the foregoing plaster of Paris mixture, the envelop is quick setting on the core and is highly porous and is insoluble in the electrolyte of the cell. In fact, the quick setting character of the dip presents some 75 difficulties from a manufacturing standpoint, in that the mixture sets relatively quickly in the dipping vessel, thereby causing some waste of material. I have discovered that these difficulties can be overcome 80 by the addition to the dip of a suitable salt to act as a retarder to the setting of the plaster.

*Plaster and salt.*—A suitable dipping magma may consist of 225 grams of plaster 85 of Paris and 225 cubic centimeters of 2% sodium borate solution. The sodium borate acts as a retarder to delay setting of the magma. For example, a plaster alone which would set in five minutes in the dipping vessel can be so retarded by the addition of a small amount of borax that it will not set for ten to twenty hours. In a thin film on the cores, however, it will set in 95 one hour, and this is rapid enough for commercial practice. Analogous salts of boric acid can likewise be used, and even other salts, so long as they would not be harmful in the battery. I have found that sodium borate is entirely harmless.

*Plaster and colloidal suspensions.*—As a substitute for sodium borate or other salt to retard the setting of the plaster dip, I may use colloidal suspensions such as starch, agar agar and the like. In addition to prolonging the time of setting, these colloidal suspensions give certain desirable characteristics to the finished cell. For instance, starch when acted on by zinc chlorid has the property of swelling or expanding. If it is incorporated into the core coating with the plaster, it remains intact while the core is out of contact with the electrolyte. When the electrolyte is poured around the core, the zinc chlorid of the electrolyte gradually attacks 115 the starch and expands the particles. This breaks up or shatters the core coating and allows a more intimate contact between the cathode mix and the electrolyte. This breaking up does not take place until after the 120 paste has gelatinized or set, and consequently there is no danger that this rupture of the plaster coating will allow carbonaceous material or manganese depolarizer to pass over into direct contact with the zinc.

A mixture that I have found to give satisfactory results consists of 500 grams plaster and 700 cubic centimeters of a 2% starch solution. Or, I may use a magma consisting of 250 grams starch, 225 grams plaster and 130

650 cubic centimeters of 2% borax solution. As another example, I may use 20 grams plaster and 50 grams of starch suspended in 100 cubic centimeters of a 10% dextrin solution.

5 Other colloids will act similarly with other electrolytes, but the use of starch to be acted on by zinc chlorid in shattering the hardened dip is the embodiment preferred by me.

10 When agar agar is used as the colloidal suspension to prolong the time of setting, this shattering of the coating does not take place, for agar agar is inert with respect to the electrolyte. It does, however, produce a 15 semi-permeable membrane which allows the transfer of ions, and with certain electrolytes and under certain conditions it may be desirable to have such a semi-permeable membrane rather than to have the coating 20 broken up through expansion of some of its components. As illustrative of the use of agar agar, a mixture of the following composition may here be mentioned. 500 grams plaster, as plaster of Paris; 7 grams agar 25 agar, and 700 grams water.

As a modification of the procedure above outlined, I have found that the cores can be dried in air when suspended by the carbon electrode, and, therefore, need not rest on a 30 greased plate, or on a layer of sand. This allows the coating to flow toward the bottom and harden into a nodule or enlargement as indicated diagrammatically at 11, Fig. 2. As a result, the coating is thicker on the 35 bottom or end of the cylinder than it is on the sides. This acts as a spacer and keeps the core further from the bottom of the zinc can than it would be if the coating were the same thickness throughout. If desirable, the bottom 40 can be paraffined, as explained in Burgess Patent No. 1,162,449, to prevent excessive action, but satisfactory life of the battery is obtainable without doing this.

This method of making dry cells of the 45 bag type eliminates the use of gauze, cheese-cloth or like fabric, now expensive and difficult to obtain; and likewise eliminates all of the hand labor of wrapping the cores and binding them with thread, and because of 50 the extreme thinness of the plaster film there is made available for useful purposes a considerable space which otherwise would be occupied by the inert cloth wrapping and its binder. With the gauze wrapping there is 55 danger of the entrapment of air when the paste is poured in and any bubble of entrapped air not only cuts down the effective area of the electrode, but also is liable to set up local actions of an undesired character.

60 With the smooth plaster film, there is no danger of air entrapment. The thickness of the film, being dependent on the viscosity of the magma into which the core is dipped, is under easy control, particularly when a retarder is used to delay setting of the dip.

A good contact is assured between the electrolyte and the cathode, and this is particularly the case when starch is incorporated in the coating, and by swelling under the action of the zinc chlorid shatters the coating after 70 the electrolyte has set to a consistency to hold the mix in position whether the coating is or is not present.

In practising the process above described and hereinafter claimed, various materials 75 may be used for the dip and for the retarder and as a means for ultimately shattering the core, and I contemplate such changes in the process and in the materials used as reasonably come within the spirit and scope of the 80 present invention as defined by the claims appended hereto.

I claim:

1. The method of dry-cell manufacture which consists in forming about a carbon 85 rod a moist active mixture of carbonaceous material and depolarizer to form a fragile dry-cell core, dipping said core in a magma to form a bibulous envelop therefor, introducing said coated core into a zinc can and 90 pouring a gelatinizable electrolyte about said core; substantially as described.

2. The method of dry-cell manufacture which consists in compressing about a carbon 95 rod a moist, active mixture of carbonaceous material and manganese depolarizer to form a fragile dry-cell core, coating said core with a magma of plaster and a suitable retarder to form a slow-setting bibulous envelop thereon, introducing said coated 100 core into a zinc anode and pouring a gelatinized electrolyte about said core.

3. The method of dry-cell manufacture which consists in arranging about a carbon rod a mixture of carbonaceous material and manganese depolarizer to form a dry-cell core, coating said core with a magma of 105 plaster of Paris to which borax has been added, thereby forming a bibulous envelop on said core, introducing said coated core 110 into a zinc can and pouring a gelatinizable electrolyte about said core.

4. The method of dry-cell manufacture which consists in compressing about a carbon rod a moist, active mixture of carbonaceous material and manganese depolarizer to form a fragile dry-cell core, coating said core with a magma of plaster containing starch and a suitable retarding salt thereby forming a bibulous envelop on said core, 115 introducing said coated core into a zinc anode and pouring about said core and electrolyte adapted to swell the starch particles of said envelop.

5. The method of dry-cell manufacture 125 which consists in arranging about a carbon rod a mixture of carbonaceous material and depolarizer to form a dry-cell core, dipping said core in a magma of about the composition of 250 grams starch, 225 grams plas- 130

4  
ter of Paris and 650 cubic centimeters of 2% borax solution, introducing said coated core into a zinc anode and pouring about said core an electrolyte capable of acting on said starch; substantially as described.

5 6. In the manufacture of dry-cells, the step which consists in dipping the carbonaceous cathode in a suitable magma to form a bibulous envelop thereon, and allowing 10 the core thus formed to harden while resting on a surface of sand, in order that grains of sand may adhere to said envelop.

15 7. The method of making dry-cells which consists in dipping the molded cathode into a magma of plaster having a suitable admixture and then allowing the thin envelop thus formed to harden on the cathode, introducing the core so produced into a zinc electrode and pouring into the space between 20 the core and the zinc electrode a gelatiniz-

able electrolyte containing zinc chlorid which acts on said admixture to effect ultimately a more intimate contact between said electrolyte and said cathode, substantially as described.

25 8. The method of making dry-cells which consists in dipping the molded cathode into a magma of plaster having an admixture of starch and then allowing the thin envelop thus formed to harden on the cathode, 30 introducing the cathode into a zinc electrode and pouring into the space between the cathode and the zinc electrode a gelatinizable electrolyte containing zinc chlorid to act on the starch and thus disrupt the 35 envelop to effect a more intimate contact between said electrolyte and said cathode; substantially as described.

In testimony whereof I affix my signature.  
ARLIE WILLIAM SCHORGER.